

Feb. 20, 1945.

J. S. NACHTMAN

2,369,748

## METHOD OF BRIGHTENING ELECTROPLATED COATINGS

Filed March 30, 1942



## Inventor

*John S. Nachtmann*

Dear Sirs  
Please accept my thanks

## UNITED STATES PATENT OFFICE

2,369,748

## METHOD OF BRIGHTENING ELECTRO-PLATED COATINGS

John S. Nachtman, Youngstown, Ohio

Application March 30, 1942, Serial No. 436,784

12 Claims. (CL. 204—36)

The invention relates generally to the heat treatment of electroplated material, and more particularly to the heat treatment of strip steel electroplated with tin or tin alloys, for the purpose of brightening the coating.

Prior practice includes heat treating metal in a non-oxidizing or reducing atmosphere such as hydrogen or carbon monoxide, but where strip metal is heat treated continuously the use of such atmospheres is very expensive and requires excessively long time periods or long heat treating chambers or both. Moreover, such atmospheres are not well adapted for heat treating electroplated coatings such as tin, because of the rapid temperature changes required in the coated strip.

In order to brighten and improve the quality of the matte-like surface which is characteristic of electroplated tin coatings, in a minimum amount of space, I have determined that it is desirable to heat the coated strip rapidly and uniformly in a non-oxidizing hydrocarbon medium to a temperature just above the melting point of 449.5° F. of tin for a short time to make the tin coating molten and close the pores thereof. While still in a non-oxidizing medium and without physically contacting anything else, the coated strip is then rapidly cooled to a temperature which is below the point of solidification of tin or below about 435° F., and then the coated strip is cooled further to below the temperature at which tin will oxidize, before being exposed to the atmosphere.

A method of brightening a tin or tin alloy coating, using a heat treating medium which boils below the melting point of the coating, for pre-heating, fusing and cooling the coating, is the subject of a separate application filed by me on March 30, 1942, Serial No. 436,783, and entitled Heat treatment of electroplated strip metal.

The subject of this application is a novel method of heat treating an electroplated tin or tin alloy coating, using a heat treating medium which boils above the melting point of the coating.

It is a general object of the present invention to provide a novel method for brightening electroplated coatings of tin or tin alloys.

Another object is to provide a novel method for continuously heat treating strip electroplated with tin or tin alloys.

A further object is to provide a novel method for rapidly heating and cooling electroplated strip continuously to brighten the coating.

A still further object is to provide a novel at-

mosphere for continuously heat treating electroplated strip.

These and other objects are accomplished by vaporizing a non-oxidizing medium of one or more hydrocarbons and which boils above the melting point of the coating, passing the strip through said vaporized medium at such a rate as to momentarily melt said coating by condensation of the vaporized medium on the strip, then immediately passing the strip into a cooled liquid bath of hydrocarbon medium to solidify the coating, and then passing the strip into another cooled liquid bath of hydrocarbon medium which is a solvent for said first and second media for cooling the strip below the oxidizing temperature of said coating.

Referring to the drawing forming part hereof, the figure is a diagrammatic cross sectional view of a preferred embodiment of apparatus for carrying out the invention.

In the drawing, the strip S, which has been previously electroplated with tin and rinsed, is shown emerging from a drier 1. The strip S is heated in the drier to a temperature below the solidification temperature of about 435° F. of the tin coating, and below the oxidizing temperature of tin.

The strip S is propelled through the apparatus by suitable means (not shown) and preferably passes over a roll 2 downwardly through a seal 3 which may be of soft material such as synthetic rubber or asbestos, and then into a vertical chamber 4 formed by refractory side walls 5 and 6 and top wall 7. The chamber 4 is the fusing compartment and is filled with heated vapor of a hydrocarbon medium which boils above the melting point of tin. The medium is circulated preferably counter to the direction of travel of the strip, and due to the fact that the strip is at a lower temperature than that of the medium, the medium condenses on the surface of the strip and gives up its heat of vaporization to the strip, so as to quickly and uniformly raise the temperature of the strip and the coating thereon. The speed of travel of the strip through the chamber 4 is regulated so that the strip is in the chamber 4 only long enough to momentarily melt the coating and brighten the same.

Preferably, a heating chamber 8 for the hydrocarbon medium is formed adjacent to the fusing chamber 4, by extending the top wall 7 and providing a side wall 9. The lower part of the heating chamber 8 is filled with the hydrocarbon medium in liquid form as indicated at X, and heating pipes 10 are provided in the liquid bath

for heating the liquid hydrocarbon **X** to vaporize the same. As the hydrocarbon medium **X** is vaporized a fan **11** circulates the vapor through opening **12** in the side wall **5** into and through the fusing chamber **4** from which it reenters the heating chamber **8** through the opening **13** near the top of side wall **5**.

Instead of preheating the strip **S** in drier **1** to 435° F., the strip can be preheated in the drier to about 200° to 225° F. and then passed through the liquid hydrocarbon **X** to further preheat it to about 435° before it passes through the vaporized medium **X** in fusing chamber **4**.

Preferably, the hydrocarbon medium **X** is a saturated or unsaturated aliphatic hydrocarbon or an aromatic hydrocarbon or a mixture of two or more which boils above the melting point of the tin coating on the strip, and preferably between 450° F. and 700° F., and which does not deposit carbon film or smudge when in contact with molten tin. Saturated and unsaturated aliphatic hydrocarbons and mixtures thereof include alkanes having a carbon chain of three or more atoms, olefins, and petroleum fractions or solvents. Aromatic hydrocarbons include coal tar fractions or solvents.

Petroleum and coal tar fractions in this boiling range are light hydrocarbons as distinguished from heavy oils, and have high rates of thermal conductivity as compared with heavy oils, but do not oxidize or vaporize to any extent at room temperatures. They have high thermostability and do not decompose or crack when heated to a soldering temperature or as high as 550° F., which accounts for the fact that no smudge is left when said fractions are in contact with molten tin.

For the purposes of illustration, I will describe the use of a high boiling petroleum solvent or fraction known as Mentor-28 as the medium **X**. Mentor-28 is a petroleum fraction with boiling points in a range of 510° F. to 650° F., a flash point of approximately 255° F. and a fire point of approximately 294° F. This material has a viscosity of 4.83 centipoises at 25° C., has practically no vapor pressure or evaporation loss at 25° C., and has a gravity range between 35° to 38° A. P. I.

The fusing compartment **4** communicates at its lower end with a tank **T** having the wall **5** as one of its side walls, and a bottom wall **14** and another side wall **15**. Preferably the tank has a partition wall **16** and the wall **6** of compartment **4** extends down into the tank between the wall **5** and the partition wall **16**. Between the walls **5** and **16** the tank is filled with a liquid hydrocarbon medium indicated at **X'** which is preferably the same hydrocarbon medium as **X**, and a passage **17** through wall **5** provides communication between the liquid mediums **X** and **X'** so that the liquid level in the lower part of chamber **4** is the same as in the lower part of chamber **8**.

The strip **S** passes downwardly into the liquid hydrocarbon **X'** between cooling coils **18** on opposite sides of the strip, and the cooling coils maintain the medium **X'** at a lowered temperature so as to immediately cool the tin coating below its solidification temperature before it contacts anything. The strip then passes under a roll **19**, upwardly between cooling coils **18'** and out of the liquid hydrocarbon **X'** where it preferably passes between squeegee rolls **20** for removing the excess liquid **X'** from the surface of the strip. The cooling coils **18** and **18'** are preferably regulated to maintain the liquid **X'** at a temperature of about 130° F.

Obviously, the hydrocarbon **X'** can be a different hydrocarbon from the medium **X** and included in the group of saturated and unsaturated aliphatic hydrocarbons and aromatic hydrocarbons or mixtures thereof. If **X'** is a different hydrocarbon medium from **X**, the passage **17** is omitted so that the two baths of liquid hydrocarbons **X** and **X'** are not connected, and the media **X** and **X'** must have sufficiently different boiling points so that they can be separated by simple distillation.

Also while the vaporizing chamber **8** is shown and described as being conveniently adjacent to the fusing compartment **4**, it is obvious that the vaporizing compartment could be located remote from the fusing compartment and the vaporized hydrocarbon conducted thereto.

From the squeegee rolls **20** the strip **S** passes over a roll **21** and then downwardly into a liquid hydrocarbon medium indicated at **Y** contained in the compartment of the tank formed between walls **15** and **16**. The hydrocarbon medium **Y** is preferably a different hydrocarbon taken from the group of saturated and unsaturated aliphatic hydrocarbons and aromatic hydrocarbons and mixtures thereof, and should have a boiling point below the temperature at which tin will oxidize; and the hydrocarbon **Y** may be hexane with a boiling point somewhere between 130° F. and 160° F. Hexane is a solvent for Mentor-28 which is preferably used as the hydrocarbon medium **X** and **X'**, and is also a solvent for any other high boiling point hydrocarbons which may be used as media **X** and **X'**.

The temperature of the hexane **Y** is maintained below its boiling point preferably by cooling pipes **18''** to keep it in a liquid state and the strip **S** passes down into the liquid **Y**, under a roll **22** and upwardly out of the liquid **Y** over a roll **23**. Preferably a partition wall **24** depends from the top wall **25** of the tank into the hydrocarbon **Y** between the rolls **21** and **23** and between the downwardly and upwardly moving portions of the strip **S** in the liquid **Y**.

As the strip passes through the hydrocarbon **Y**, the film of hydrocarbon **X** and **X'** on the strip is dissolved by the hydrocarbon **Y** and as the strip leaves the hydrocarbon **Y** it passes between squeegee rolls **26** to remove excess film before the strip passes over the roll **23**.

From the roll **23** the strip passes through an opening **27** in wall **15** and into a small tank **28** containing a low boiling liquid hydrocarbon **Y'** selected from the group of saturated and unsaturated aliphatic hydrocarbons and aromatic hydrocarbons and mixtures thereof, and the strip passes through the liquid hydrocarbon **Y'** under roll **29** and then preferably through squeegee rolls **30** and out of the tank **28** through a seal **31**.

In tank **28** the liquid hydrocarbon **Y'** is preferably hexane to which about one-half per cent by weight of palm oil or other vegetable oil has been added, and the liquid **Y'** is kept at a temperature at or below room temperature preferably by cooling pipes **28'** so as to further cool the strip as it passes through the same. As the strip passes through the squeegee rolls **30** the film of liquid hydrocarbon **Y'** is spread uniformly and thinly over the strip, and as the strip emerges through the seal **31** the hexane will evaporate from the strip surface leaving an imperceptible oil film thereon. The percentage of vegetable oil added to the liquid **Y'** may be varied somewhat depending upon the thickness of oil film desired to be left on the strip surface.

AND WAVE ENERGY.

210

2,369,748

3

A distillation system of conventional design indicated at 32 may be used to separate the carry over of the liquid X' from the liquid Y. Thus the liquid Y with the carry over X' is conducted through pipe 33 to the distillation apparatus 32, from which the separated liquid X' is pumped through pipe 34 and pump 35 back to the compartment containing the liquid X'. The pure liquid Y is pumped from the distilling apparatus 32 through a pipe 36 and pump 37 to sprays 38 which spray the strip as it emerges from liquid Y to remove all traces of liquid X' and X from the surface of the strip.

If different high boiling point hydrocarbons are used for X and X', there will be a carry over of the liquid X on the strip surface into the liquid X', and a distillation system similar to that indicated at 32 can be used to separate the liquids X and X' and return them to their proper compartments.

The strip carrying rolls 2, 19, 21, 22, 23 and 29 are made of a suitable material such as polished steel, or polished chrome plated steel, which will not mar or scratch the surface of the strip, and these rolls are preferably driven at the speed of travel of the strip to prevent any marring of the surface due to slippage between the strip and the roll surface.

Liquid hydrocarbons X' and Y may be the same hydrocarbon in which case the partition wall 16 may be omitted together with rolls 22 and 23, so that the strip passes directly from roll 21 into the tank 28.

If desired, the hydrocarbon medium in any of the compartments may be introduced therein by means of sprays or jets directed against the strip.

The term "hydrocarbon medium" as used herein means a saturated or unsaturated aliphatic hydrocarbon or an aromatic hydrocarbon, or a mixture of two or more of said hydrocarbons, which boils above the melting point of tin and preferably between 450° F. and 700° F., and which does not deposit carbon film or smudge when in contact with the molten coating.

While I have described the heat treatment of electroplated strip metal, the invention may be applied to strip sheets, sheets, wire and the like, without departing from the scope of the invention as defined in the appended claims.

I claim:

1. The method of heat treating material electroplated with a coating of tin, which includes vaporizing a petroleum fraction which boils between about 450° F. and 700° F., passing the material through said vaporizing petroleum fraction at such a rate as to momentarily melt said coating by condensation of said petroleum fraction on said material, and then passing the material immediately into a cooled liquid bath of hydrocarbon medium to solidify the coating.

2. The method of heat treating material electroplated with a coating of tin, which includes vaporizing a petroleum fraction which boils between about 450° F. and 700° F., passing the material through said vaporized petroleum fraction at such a rate as to momentarily melt said coating by condensation of said medium on said material, and then passing the material immediately into a cooled liquid bath of said petroleum fraction maintained at a temperature of about 130° F.

3. The method of heat treating material electroplated with a coating of tin, which includes vaporizing a coal tar fraction which boils between about 450° F. and 700° F., passing the ma-

terial through said vaporized coal tar fraction at such a rate as to momentarily melt said coating by condensation of said coal tar fraction on said material, and then passing the material immediately into a cooled liquid bath of hydrocarbon medium to solidify the coating.

4. The method of heat treating material electroplated with a coating of tin, which includes vaporizing a coal tar fraction which boils between about 450° F. and 700° F., passing the material through said vaporized coal tar fraction at such a rate as to momentarily melt said coating by condensation of said medium on said material, and then passing the material immediately into a cooled liquid bath of said coal tar fraction maintained at a temperature of about 130° F.

5. Improvements in the plating of metals which comprise electrolytically depositing a coating of tin on a ferrous strip, and then continuously passing the metal coated strip thru the vapor of a petroleum hydrocarbon having a boiling point above the melting point of tin until the coating of tin is raised to a temperature above its melting point by condensation of said hydrocarbon vapor on the tin surface.

6. The method of heat treating material electroplated with a coating of tin for brightening the tin surface, which includes vaporizing a first hydrocarbon medium which boils above the melting point of tin, exposing the material to said vaporized medium to momentarily melt said coating and brighten the same by condensation of said first medium on said material, then immediately passing the material into a cooled liquid bath of a second hydrocarbon medium to solidify the coating, and then passing the material into a cooled liquid bath of a low boiling hydrocarbon medium which is a solvent for said first and second media.

7. The method of heat treating material electroplated with a coating of tin, which includes vaporizing a hydrocarbon medium which boils between about 450° F. and 700° F., passing the material through said vaporized hydrocarbon medium at such a rate as to momentarily melt said coating by condensation of said hydrocarbon medium on said material, then passing the material immediately into a cooled liquid bath of hydrocarbon medium to solidify the coating, and then passing the material into a cooled liquid bath of hydrocarbon medium which dissolves the film of hydrocarbon medium left on the surface of said material.

8. The method of heat treating material electroplated with a coating of tin, which includes vaporizing a hydrocarbon medium which boils between about 450° F. and 700° F., passing the material through said vaporized hydrocarbon medium at such a rate as to momentarily melt said coating by condensation of said medium on said material, then passing the material immediately into a cooled liquid bath of said hydrocarbon medium maintained at a temperature of about 130° F., and then removing the film of said hydrocarbon medium from the surface of the material.

9. The method of continuously heat treating ferrous strip electroplated with a coating of tin, which includes vaporizing a hydrocarbon medium which boils between about 450° F. and 700° F., passing said strip through said vaporized hydrocarbon medium at such a rate as to momentarily melt said tin coating by condensation of said medium on said strip, and then passing the strip immediately into a cooled liquid bath of

said hydrocarbon medium to solidify the coating.

10. The method of continuously heat treating ferrous strip electroplated with a coating of tin, which includes vaporizing a hydrocarbon medium which boils between about 450° F. and 700° F., passing said strip through said vaporized hydrocarbon medium at such a rate as to momentarily melt said tin coating by condensation of said medium on said strip, and then passing said strip immediately into a cooled liquid bath of said hydrocarbon medium maintained at a temperature of about 130° F.

11. Improvements in the plating of metals which comprise electrolytically depositing a coating of tin on a metal base stock and then continuously passing the metal coated stock thru the vapor of a hydrocarbon medium having a boil-

ing point above the melting point of tin until the coating of tin is raised to a temperature above its melting point by condensation of the said hydrocarbon vapor on the tin surface.

12. Improvements in the plating of metal 5 which comprise electrolytically depositing a coating of tin on a metal base stock, then continuously passing the metal coated stock thru the vapor of a hydrocarbon medium having a boiling point above the melting point of tin until the coating of tin is raised to a temperature above its melting point by condensation of said hydrocarbon vapor on its surface, and then immediately passing the strip thru a liquid bath of hydrocarbon medium maintained at a temperature of about 130° F. to solidify the tin.

JOHN S. NACHTMAN.